

March 2, 1965

V. C. SICKLE ET AL

3,171,151

CLEANING AND POLISHING ARTICLE

Filed April 4, 1961



INVENTORS:

V. Claude Sickle  
Herbert W. Schnabel  
Julian J. Cibular

By Carl C. Batz, Attorney

1

3,171,151

**CLEANING AND POLISHING ARTICLE**

Vernon Clyde Sickle, Herbert W. Schnabel, and Zoltan J. Cibulas, Alliance, Ohio, assignors to Armour and Company, Chicago, Ill., a corporation of Delaware  
Filed Apr. 4, 1961, Ser. No. 100,764  
4 Claims. (Cl. 15—118)

The present invention relates to improved fibrous articles finding special utility in the maintenance of floors and to the method of making such articles.

In the maintenance of floors, attempts have been made to utilize pads formed of animal, vegetable, mineral and synthetic fibrous materials bonded together by a suitable binder material and incorporating abrasive grains distributed throughout the fibrous pad.

Several difficulties arise in the use of such pads. In floor cleaning operations, aqueous solutions of such chemicals as caustic potash, ammonia, trisodium phosphate and the like are commonly used. Such solutions cause a rapid loss in the tensile strength, compression set and load deflection of these fibrous pads. This problem is particularly evident when animal fibers are utilized. The incorporation of abrasive particles such as silicon carbide in such floor maintenance articles is of benefit where an aggressive action is required. However, such floor maintenance articles incorporating abrasive grits cannot be used in the polishing of floors.

Accordingly, it is an object of the present invention to provide an improved fibrous article for use in floor maintenance operations not subject to the above-mentioned shortcomings and difficulties.

It is a further object of this invention to provide an improved fibrous article useful in the maintenance of floors which can be used both in cleaning and polishing operations in the maintenance of floors.

Further and additional objects of this invention will become apparent from the following specification in the accompanying drawings in which:

FIG. 1 is a partial diagrammatic view of a production line for producing the fiber pad of this invention; and

FIG. 2 is a perspective view of a fiber pad embodying this invention; and

FIG. 3 is a sectional view of our improved fiber pad taken on the line 3—3 of FIG. 2.

In accordance with the present invention, we provide a stereoreticulate mass of curled organic fibers of substantially uniform thickness in the form of a pad. The fibers of the pad are firmly bonded together at points where they cross and contact one another by a vulcanized binder or elastomer. The fibers are also provided with a coating of a water-repellant material. The fiber pad of this invention performs a dual function. That is, it can be used both in the cleaning and polishing of floors. In such a pad one operable side of the pad is more aggressive, of greater density and of less resiliency than the opposite side of the pad.

The organic fibers used as a starting material in accordance with the present invention include the common types of commercial animal hair, such as horse hair, cattle hair, and hog hair. Specifically desirable types of animal hair from both an economic and functional standpoint are relatively short hairs, such as hog hair. However, longer types of hair, such as cattle tail hair, horse mane hair, etc., can also be employed. Excellent results are obtained with hog hair which can contain a percentage of other types of hair, such as cattle tail hair. Preferably, the hair fibers have an average diameter of from about 2.0 to about 9.0 mils. Synthetic fibers such as "nylon" and "dacron" can also be utilized. The fibers employed preferably have a three dimensional curvature impressed

2

upon them by a curling or crimping process. Such curling or crimping can be accomplished by mechanical means or by the more recently developed chemical curling processes. The curling or crimping of the fibers by either mechanical or chemical means introduces a three dimensional curl or crimp in the fibers so that a random distribution of the fibers on a flat surface produces an approximate stereoreticulate mass.

The initial step in the production of the fiber pads involves the spreading of the curled organic fibers in a layer of the desired thickness. This can be accomplished mechanically and the fibers are allowed to fall on a horizontal surface so that it assumes a random distribution and forms a fibrous mat or web of a predetermined bulk density. For the preparation of pads used in floor maintenance operations, a finished web or pad from three quarters to two inches in thickness is preferred.

Referring to FIG. 1 of the drawing, there is shown in diagrammatic form the apparatus for carrying out the production of the floor maintenance pads. The curled fibers, for example, curled animal hair in hopper 10 is fed downwardly onto a slide 11 from which it is discharged into a fiber spreader 12. In FIG. 1 as illustrated, the fiber spreader 12 is equipped with wiretoothed carding cylinders 13 and 14, which separate the fibers as they are discharged from the slide 11. The fiber spreader 12 also includes two lower spreading rolls 15 and 16. The fluffy mass of fibers 17 is discharged downwardly by the carding rolls 13 and 14 and spreading rolls 15 and 16 onto a continuous conveyor belt 20 where it is formed into a web 18 of any desired thickness.

Following the formation of the flat fibrous mat or web, the web 18 passes beneath an interlacer 21. This interlacer is provided with a series of needlelike members 22, which needle members operate in a vertical plane and penetrate into the web 18. This operation serves to compact the upper portion of the web or pad 18 and it is preferable that the needles penetrate to a depth of about three-fourths of the thickness of the web. Thus in the upper portion of the web the fibers will be of greater density than the lower portion of the web. This upper portion by having a greater fiber density, is also less resilient than the lower half of the pad and is useful in scrubbing or cleaning operations.

Following the interlacing operation, the fiber mat or web 18 is sprayed with an elastomer for the purpose of bonding the fibers together. With webs of about three-fourths (3/4) to two (2) inches in thickness, it has been found desirable to spray the web a single time from each side. This gives best penetration by the liquid elastomer dispersion and prevents the dispersion from collecting on the conveyor or other supporting surface.

Referring again to FIG. 1 of the drawings, the web 18 is shown being carried toward the right from the interlacer 21 by conveyor belt 20 to a spraying station or zone 23 wherein one side of the web is sprayed with the liquid elastomer dispersion. In the illustration as shown, there is a spray head 24 which is preferably of the oscillating type so that it moves back and forth across the web during the spraying operation. Sufficient elastomer is applied at spray station 23 to penetrate the upper half of the web. Thereafter, conveyor belt 20 takes the partially elastomer-coated web through a dryer zone 25 wherein the elastomer coating is dried to an indispersible but unvulcanized condition. This operation increases the tensile strength of the mat so that it can be inverted without tearing and also so that the elastomer coating will not drain downwardly upon the conveyor belt when the web is inverted and cause the web to stick. The time required in the dryer zone 25 will be between about 15 to 20 seconds when the dryer

of the hot air blast type is utilized. The partially coated web 18 is then passed through a series of rollers 26 where the upper portion of web 18 is further compacted and densified.

The partially coated web 18 is then taken over an inverter 27 which turns the web over so that the uncoated portion of the web or mate is now uppermost on the conveyor 20. The mat is then conveyed through a second spraying zone 28 similar to spraying zone 23. If desired, it, too, can be equipped with an oscillating spray head 29 of the same type as spray head 24. Sufficient elastomer is applied in this spray station 28 to penetrate to the center of the web and thus complete the distribution of the elastomer throughout the web.

After the web 18 has been sprayed at station 28 it is passed through a curing oven 31 where the elastomer used to bond the fibers together is cured. The temperatures employed in this curing oven are in the range of about 260° F. to 325° F. for from 4 to about 10 minutes depending on the elastomer.

From the curing oven 31 the vulcanized web 18 is passed under a cutting press 32 wherein the continuous web 18 is die cut into pads of various shapes, such as discs.

Following the cutting operation, the vulcanized pads are conveyed into tank 33 containing a suitable water-repellant solution. The fiber pad is soaked in the solution for a period from 2 to 10 minutes, then removed, allowed to drain, and then conveyed on to oven 34 to remove any volatile solvent and to dry the pad.

Various types of elastomer dispersions or binders can be employed in this invention. It is preferred to employ an aqueous dispersion of a vulcanizable elastomer. The elastomer can be either a natural rubber or latex, a synthetic elastomer latex, or a reclaimed rubber dispersion. The rubber or synthetic elastomer dispersion is compounded with other ingredients to facilitate the application in curing of the elastomer. Water may be added to secure the required consistency for application. Specific examples of elastomers which can be employed include natural rubber, butadiene-styrene dispersions, neoprene rubber dispersions, polyvinyl chloride, etc. Typical formulae of such compounded vulcanizable elastomers are set out in Table I below:

TABLE I

|                                    | Formula A<br>(Dry Parts) | Formula B<br>(Dry Parts) | Formula C<br>(Dry Parts) | Formula D<br>(Dry Parts) | Formula E<br>(Dry Parts) |
|------------------------------------|--------------------------|--------------------------|--------------------------|--------------------------|--------------------------|
| Neoprene 842A                      | 70.00                    | 70.00                    | 51.00                    | 51.00                    |                          |
| Natural Latex                      |                          |                          |                          |                          |                          |
| Naug. 2714                         | 30.00                    | 30.00                    | 15.00                    | 15.00                    |                          |
| Nekal A                            | 0.40                     | 0.40                     | 1.00                     | 1.00                     |                          |
| Casein                             | 0.60                     | 0.60                     | 0.51                     | 0.51                     |                          |
| Ammonia                            | 0.84                     | 0.84                     | 0.31                     | 0.31                     |                          |
| Tepidone                           | 0.35                     | 0.35                     |                          |                          |                          |
| Clay                               | 45.20                    |                          | 46.90                    |                          |                          |
| Silica Flour                       | 9.68                     | 75.0-125.0               |                          | 75.0-125.0               |                          |
| Darvan #2                          | 1.72                     | 1.72                     | 1.25                     | 1.25                     |                          |
| Caustic Potash                     | 0.15                     | 0.15                     | 0.40                     | 0.40                     |                          |
| Zinc Oxide                         | 17.31                    | 17.31                    | 4.25                     | 4.25                     |                          |
| Sulfur                             | 0.60                     | 0.60                     | 3.30                     | 3.30                     |                          |
| Agerite White                      | 0.67                     | 0.67                     | 0.85                     | 0.85                     |                          |
| Antioxidant 2246                   | 0.35                     | 0.35                     |                          |                          |                          |
| Butyl Zinat                        | 0.85                     | 0.85                     |                          |                          |                          |
| Aquarex D                          |                          |                          | 0.83                     | 0.83                     |                          |
| Setsit 5                           |                          |                          | 0.43                     | 0.43                     |                          |
| GRS 2000                           |                          |                          | 34.00                    | 34.00                    |                          |
| Agerite Resin D                    |                          |                          | 0.85                     | 0.85                     |                          |
| Captax                             |                          |                          | 0.85                     | 0.85                     |                          |
| Darvan #1                          |                          |                          | 0.64                     | 0.64                     |                          |
| Polyvinyl chloride<br>(Geon 576)   |                          |                          |                          |                          | 100.00                   |
| Acrotex M3                         |                          |                          |                          |                          | 43.00                    |
| Aerotex AS                         |                          |                          |                          |                          | 13.00                    |
| Silican Carbide (Grade<br>180-600) |                          |                          |                          |                          | 155.00                   |
| Triton X-100                       |                          |                          |                          |                          | 0.20                     |
| Carbon black                       |                          |                          |                          |                          | 3.00                     |

As shown in FIG. 1, the water-repellant coating is applied to the fiber pad after the pad has been completely sprayed with the suitable elastomer and passed through the curing oven. However, the water-repellant materials

may be also used to treat the fibers prior to the application of any elastomer material.

As an alternate procedure, the water-repellant material may also be admixed in the latex or elastomer material and applied in the spraying zones 23 and 28.

Table II below lists examples of various water-repellant compositions which can be utilized in this invention:

TABLE II

| 10 | Water Repellant Material                                                                                                                                                                                   | Comment                                                                                                                                                                             |
|----|------------------------------------------------------------------------------------------------------------------------------------------------------------------------------------------------------------|-------------------------------------------------------------------------------------------------------------------------------------------------------------------------------------|
| 15 | 1. 10% aluminum Formate Solution.<br>2. 3% Solution of Arquad 2HT-75<br>3. 5% Solution of Dow Silicone D-772.<br>4. 10% Solution of Aerotex M-3.<br>5. 10% Solution of Aerotex AS.                         | These materials are especially suitable for treating the fibers prior to the application of any elastomer material.                                                                 |
| 20 | 6. Paraffin Wax Emulsions:<br>(a) Ceremul A-Naugatuck Sun Bloom Wax.<br>(b) Carbonwax.<br>(c) du Pont Helizone Wax.<br>(d) Cermul Q.                                                                       | These wax materials are particularly suited for incorporation in the latex or elastomer material. For this purpose, about 5-15 parts of wax per 100 parts of dry elastomer is used. |
| 25 | 7. One part of Street REP-100 dissolved in 6 parts of Stoddard Solvent.<br>8. 10% solution of 3MFC 805 (This material is composed of 30% Fluorochemical, 60% Isopropyl Alcohol, 5% water and 5% Chromium). | This material is suitable for treating the elastomer vulcanized pad.                                                                                                                |
| 30 | 9. 10% solution of du Pont Zelan FF.<br>10. 10% solution of du Pont Zelan AP.<br>11. 10% solution of du Pont Quilon Chrome Complex.                                                                        | The treated pad is dried in an oven for about 10 minutes at 250° F.                                                                                                                 |
| 35 |                                                                                                                                                                                                            | The pads are placed in these solutions for about 10 minutes and dried at 250° F. for about 10 minutes.                                                                              |

Not only does the treatment of the pad with the water repellent materials dramatically improve the life of the fiber pad when the pads are used in floor cleaning and scrubbing operations, but we have also discovered that the water repellancy treatment more completely channels the aqueous cleaning solutions used in floor maintenance operations through the pad, thus serving the distribute the solution to all the fibers resulting in a more thorough cleaning action. Additionally, this also functions in better cleansing of the pad itself.

FIGS. 2 and 3 of the drawings illustrate a preferred embodiment of this invention. The fibers in the upper portions 41 of this pad 40 are denser, less resilient and

more aggressive than are the fibers in the lower portion 42 of the pad. In floor maintenance operations the pad 40, which is shown in perspective in FIG. 2, is mounted to any conventional rotary floor maintenance machine.

When it is desired to use this dual function pad in floor cleaning or scrubbing, side 41 of the pad is mounted so as to be in contact with the floor surface. Correspondingly, if the pad is to be used in the polishing of floors, then the pad is mounted so that side 42 of pad 40 is in direct contact with the floor surface.

The invention can be further illustrated by the following examples:

*Example I*

A web of curled animal hair fibers weighing approximately 4 ounces per square foot and comprising 80% hog hair and 20% cattle tail hair was formed on a conveyor. The mat or web of curled hair was passed beneath an interlacer so adjusted that the needle penetration was approximately three-fourths (¾) of the thickness of the mat. Following the interlacing operation, the mat was sprayed with an aqueous dispersion of a neoprene rubber composition prepared according to Formula B, of Table I. Following the application of the elastomer, the mat was passed through a drying zone for about 20 seconds wherein a blast of hot air was directed over the mat to set the elastomer.

Thereafter, the partially coated mat was passed through a series of rollers to further compact and densify the upper portion of the mat.

The mat was then turned over so that the uncoated portion was uppermost on the conveyor and sprayed with an aqueous dispersion of a neoprene rubber composition prepared according to Formula A, of Table I. Thereafter, the sprayed mat was conveyed into a curing oven for about 6 minutes at approximately 290° F.

A series of discs (12 inches in diameter) was cut from the continuous mat and passed into a tank containing a solution of a water-repellant material. This water-repellant material consisted of one part of Street REP-100 dissolved in 6 parts of Stoddard solvent. The fiber discs remained in the water-repellant solution for about 6 minutes, removed, allowed to drain and thereafter conveyed through an oven to remove any volatile solvent and to dry the pad. The finished pad had a thickness of 1.25 inches and weighed approximately 8 ounces per square foot.

*Example II*

Fiber pads were made in the same manner as in Example I with the exception that an aqueous dispersion of a natural rubber composition prepared according to Formula C, Table I, was sprayed on the side of the mat wherein the fibers had been previously densified by inter-

lacing. The opposite side of the mat was sprayed with an aqueous dispersion of a natural rubber composition prepared according to Formula D, Table I.

While in the foregoing specification this invention has been described in considerable detail, it will be apparent to those skilled in the art that many of the specific details and embodiments can be varied widely without departing from the broad idea of the invention.

We claim:

- 10 1. A cleansing and polishing article comprising a stereoreticulate mass of curled organic fibers in the form of a reversible pad of substantially uniform thickness having two opposed operable sides, said fibers being bonded together at points where they cross and contact one another by a vulcanized elastomer, one operable side of said pad being of uniformly greater fiber density and of less resiliency than the opposite operable side of said pad.
- 15 2. A cleansing and polishing article comprising a stereoreticulate mass of curled organic fibers in the form of a pad having two opposed operable sides, said fibers being bonded together at points where they cross and contact one another by vulcanized elastomer, one operable side of said pad being of greater density and of less resiliency than the opposite operable side of said pad, said fibers having a coating of a water-repellant material.
- 20 3. The article of claim 2 wherein said water-repellant material is incorporated into said vulcanized elastomer.
- 25 4. A cleansing and polishing article comprising a stereoreticulate mass of curled hair fibers in the form of a reversible pad of substantially uniform thickness and having two opposed operable sides, said fibers having a coating of a water-repellant water and being bonded together at points where they cross and contact one another by a vulcanized elastomer, one operable side of said pad being of greater density and of less resiliency than the opposite operable side of said pad.
- 30 35

References Cited in the file of this patent

UNITED STATES PATENTS

|    |           |                     |               |
|----|-----------|---------------------|---------------|
| 40 | 1,334,744 | Farr -----          | Mar. 23, 1920 |
|    | 1,873,030 | Quinn -----         | Aug. 23, 1932 |
|    | 2,375,585 | Rimer -----         | May 8, 1945   |
|    | 2,526,468 | Frye -----          | Oct. 17, 1950 |
| 45 | 2,803,577 | Colt et al. -----   | Aug. 20, 1957 |
|    | 2,958,593 | Hoover et al. ----- | Nov. 1, 1960  |

FOREIGN PATENTS

|         |               |               |
|---------|---------------|---------------|
| 181,389 | Austria ----- | Mar. 10, 1955 |
|---------|---------------|---------------|